

July 11, 1967

J. Y. WELSH

3,330,649

UPGRADING MANGANESE ORES USING HF AND  $H_2SiF_6$  AS  
LEACHING MATERIALS  
Filed May 27, 1964



# United States Patent Office

3,330,649

Patented July 11, 1967

1

3,330,649

## UPGRADING MANGANESE ORES USING HF AND H<sub>2</sub>SiF<sub>6</sub> AS LEACHING MATERIALS

Jay Y. Welsh, Catonsville, Md., assignor to Manganese Chemicals Corporation, Baltimore, Md., a corporation of Minnesota

Filed May 27, 1964, Ser. No. 370,569  
6 Claims. (Cl. 75—101)

This invention relates to the art of hydrometallurgically 10 beneficiating manganese ores whose manganese content is largely in the form of manganese dioxide, and is concerned with the upgrading of ores which are relatively high in MnO<sub>2</sub> but which contain significant amounts of silica and other impurities. The invention is particularly 15 concerned with the provision of a cyclical process of upgrading such ores with simultaneous production of certain by-products having substantial economic value. The invention has both process and product aspects.

By the expression "manganese ores relatively high in 20 MnO<sub>2</sub>" are here meant ores whose content of MnO<sub>2</sub> amount to at least 50% by weight of the total.

Manganese ores almost invariably contain at least some Mn<sup>+2</sup> and Mn<sup>+3</sup>. Also, they contain silica in greater or lesser amount together with measurable amounts of alumina and of at least one compound of at least one member (or, usually, of a plurality of members) of the metals group consisting of Fe, Pb, Zn and Cu and sometimes an oxidic compound of an alkali or/and alkaline earth metal. In the specific examples appearing hereinbelow 30 there are set out partial analyses (limited to manganese and those impurities occurring in more substantial amounts) of several representative "manganese ores relatively high in MnO<sub>2</sub>." In this connection, it should be noted that (1) some of the frequently encountered impurities in manganese ores are present amongst the "gangue" components of the ore, while (2) some of them are "built" into the manganese dioxide crystal. Generally speaking, alkali oxides and up to about 5.0% Fe and up to about 0.7% Pb and smaller amounts of Cu, Zn, P and As are (or appear to be) incorporated in the MnO<sub>2</sub> structure. As will be brought out hereinbelow, impurities of the "1" type above are amenable to the upgrading process of the present invention, whereas some of the impurities of the "2" type are relatively very poorly removable by the process.

In its broader aspect, the upgrading process of the present invention comprises treating an ore, of the composition above described, in particulate form, with an aqueous solution of a dissolving agent of the group consisting of HF, H<sub>2</sub>SiF<sub>6</sub> and mixtures of HF and H<sub>2</sub>SiF<sub>6</sub> whereby to extract or leach out non-MnO<sub>2</sub> components of the ore which are soluble in such solution (pure MnO<sub>2</sub> is not soluble in such solution), and separating the resulting liquid phase (containing fluorine values in the form of silicofluorides and hydrofluoric acid, and solubilized impurities leached from the ore), and the resulting solid phase, i.e., the upgraded ore, by conventional separatory measures e.g., decantation, filtration, and the like. The aforesaid treating step may be carried out in a leach column containing more or less coarse MnO<sub>2</sub> ore particles (e.g., particles from one-fourth inch diameter to particles as small as 6 mesh or smaller); or, the par-

2

ticulate ore may be slurried with the above-described liquid treating agent, in which latter event the maximum particle size is determined by its slurryng ability.

Since SiO<sub>2</sub> and Al<sub>2</sub>O<sub>3</sub> almost always are encountered 5 in the ore, the treating agent includes both hydrofluosilicic acid and hydrofluoric acid, since the latter is needed for decomposing the SiO<sub>2</sub> and to assist in the breakdown of the Al<sub>2</sub>O<sub>3</sub>. The reaction of HF with SiO<sub>2</sub> produces SiF<sub>4</sub> which becomes solubilized as H<sub>2</sub>SiF<sub>6</sub>. The aforesaid separated aqueous phase contains, then, the so-formed H<sub>2</sub>SiF<sub>6</sub> and the solubilized metals: apparently, any solubilized iron, lead, zinc, copper and Mn<sup>+2</sup> and Mn<sup>+3</sup> values are present as silicofluorides, and the aluminum probably as complex silicofluorides.

In connection with the above-described process, it is to be noticed that all of the solubilized metal silicofluorides can, if so desired, be recovered; also, that fluorine values can be regenerated. Whatever HF becomes "used up" in decomposing SiO<sub>2</sub> represents the extent to which H<sub>2</sub>SiF<sub>6</sub> "builds up" in said "liquid phase," and hence part of the H<sub>2</sub>SiF<sub>6</sub> content can be separated from the liquid phase as a by-product having economic value.

As will, then, be appreciated, the principles of the present invention quite naturally find economic expression 25 in a cyclic process in which (a) raw ore and make-up HF are continuously or intermittently added to the closed circuit, and (b) upgraded ore and by-product H<sub>2</sub>SiF<sub>6</sub> are continuously or intermittently removed from the circuit. The hereinabove-described general process is integrated into the cyclic process, which latter may be described as follows:

Particulate MnO<sub>2</sub> ore (of the gangue-containing kinds described hereinbefore) and an aqueous solution of H<sub>2</sub>SiF<sub>6</sub> and HF are continuously introduced into a dissolving 35 zone to leach out the ore, more or less completely, gangue constituents of such ore thereby yielding a solid phase consisting essentially of upgraded MnO<sub>2</sub> ore and a liquid (aqueous) phase containing metal silicofluorides (derived from impurities in the raw ore), the introduced H<sub>2</sub>SiF<sub>6</sub> and additional H<sub>2</sub>SiF<sub>6</sub> (derived from the SiO<sub>2</sub> decomposed out of the raw ore). The solid and liquid phases are continuously separated from each other, and the solid phase may be and preferably is washed to a reasonable extent, and is withdrawn from the circuit as product (upgraded) 40 MnO<sub>2</sub> ore. A part of the liquid phase is recycled to the dissolving zone, while the remainder of the separated liquid phase is continuously treated with a fluosilicate-decomposing agent so as to regenerate, from the soluble silicofluorides contents of the liquid phase, H<sub>2</sub>SiF<sub>6</sub> in the form of an aqueous solution suitable for recycling to the dissolving zone. The "additional" H<sub>2</sub>SiF<sub>6</sub> which had been derived from the SiO<sub>2</sub> content of the raw ore may be, and preferably is, withdrawn from the circuit as by-product H<sub>2</sub>SiF<sub>6</sub>. The "by-product H<sub>2</sub>SiF<sub>6</sub>" desirably should 45 equal in amount the make-up HF plus the silica leached from the raw ore. Preferably, the silicofluoride and fluoride-decomposing agent is sulphuric acid (e.g., H<sub>2</sub>SO<sub>4</sub> of about 70% concentration), and in this decomposing step the metal silicofluorides (of the liquid phase) preferably are converted to metal sulphates. To the extent that Mn<sup>+2</sup> and/or Mn<sup>+3</sup> values (present in the raw ore) had been solubilized and carried in the aforesaid "liquid phase," this manganese will—through the reaction with H<sub>2</sub>SO<sub>4</sub>—be 50 55 60

converted to manganese sulphate, and the latter may be recovered and put to use either as such or as starting material for preparing manganese metal or some other manganese compound. For recovering these manganese values I may treat the still bottoms sludge with  $MnO$  and  $H_2O$  and adjust the pH to 5.0-5.5, at which point Fe and Al values precipitate leaving an aqueous phase consisting largely or wholly of a solution of  $MnSO_4$ . While such recovery of Mn values from the still bottoms sludge is not a necessary step in my cyclic process, it has such economic or technological worth as to be included in any actual processing plant flow sheet, such for illustrative purposes as the sole figure of the appended drawing.

The liquid-vapor equilibria within the distilling column impose the most basic theoretical limit on composition. These data dictate that the free HF in the recycle liquor should not exceed 5% (and preferably not more than 3%) if HF losses are to be avoided in the water balance, and that the  $H_2SiF_6$  concentration in the recycle liquor cannot exceed 41 to 43% (depending on the HF concentration). Values ought not to be exceeded, since a water balance by means of a distilling column otherwise would be impossible.

The method of maintaining water balance is of basic importance in defining the process. Otherwise most of the fluoride values would have to be discarded, with poor economics, or complicated and expensive reclaiming processes would have to be employed. With the process as defined, operated in an optimum manner, water balance is maintained by volatilization, i.e., all of the excess wash water (over that required for the 30%  $H_2SiF_6$  by-product) is removed from the top of the distillation column. All metals leached are removed as sludge sulfates with a minimum of concentrated (70%)  $H_2SO_4$ .

The beneficiation effected on most commercial, large volume, Mn ores is outstanding. A common metallurgical grade ore can easily be upgraded to far surpass the best chemical grade ores.

In my complete cyclic process, that which "cycles" is the majority of the dissolving agent ( $H_2SiF_6$  and HF, in aqueous solution) which is present in excess. The particulate ore passes into and out of the closed circuit, as does the wash water. The HF which is (continuously or intermittently) added as "make-up HF" departs from the circuit in the  $H_2SiF_6$  by-product. The added  $H_2SO_4$  departs as sulphates and waste free acid in the still bottoms sludge. In the still itself there is eliminated the water which entered the circuit as wash water, less that amount of water which goes out in the 30% solution of  $H_2SiF_6$  by-product and less the small amounts which depart the circuit in the  $MnO_2$  product filter cake and in the still bottoms sludge.

The process of the present invention will now be described in greater particularity and with reference to the accompanying drawing, in which

The single figure is a flow sheet of the complete process.

In the drawing, 1 represents a reaction vessel provided with an agitator means 2. Raw ore is fed to the reaction vessel as at 3, while a solution of  $H_2SiF_6$  is delivered to the vessel through pipe 4 and make-up HF is delivered as at 5. A heat-exchange means 6 is installed in reaction vessel 1 to maintain the temperature of the reaction mixture at, say, about 90° C.

Reaction mixture slurry is transferred from vessel 1, by means of pump 8 and conduit 10, to a thickener 11 of known type, wherein the solids content of the slurry is countercurrently washed with water admitted through pipe 12. Effluent from the thickener is transferred, through pipe 20 to places of use (to be described hereinbelow), whilst the partially thickened solids are pumped, by pump 13 to the next in series of a series of generally similar thickeners, e.g. six, more or less, wherein the solids are washed free from hydrofluoric acid, hydroflu-

silic acid, and salts of hydrofluosilicic acid, and the wash waters are combined, for the recovery of values. After the washing has been carried out to an acceptable pure solids product, the resulting partially dewatered slurry of particulate  $MnO_2$  is delivered through conduit 15 to a filter 16. The resulting filter cake is conventionally dried, whereupon it is in merchantable form. The resulting filtrate is or may be discarded.

A part of the effluent from the thickeners is passed—by means of valved conduit 21a—to the reaction vessel. The remainder of said effluent is passed—by means of valved conduit 21b—to the agitator equipped boiler section 22 of a recycle still wherein it is maintained at an elevated temperature of about 165° C. by conventional indirect heat exchange means, and is reacted with concentrated  $H_2SO_4$  (admitted through conduit 40), to decompose the contents of metal salts of hydrofluosilicic acids to yield the free acid and sulphates of said metals. The overhead product passes into the upper—refluxing—section 23 of the recycle still, in which latter section the vapor is contacted, in the packed column part 24 of section 23, with cooling liquid admitted through coolant line 25. Steam is discharged at 26, whilst a hydrofluoric acid-containing solution of hydrofluosilicic acid accumulates in the base 27 of this section. Said concentrate is withdrawn by pump 28 and line 29, and is delivered partly to valved hydrofluosilicic acid solution make-up line 4—for use in reaction vessel 1—and partly to a valved line 30 for delivery to a neutralizing vessel 31 equipped with agitating means 32. In vessel 31 the hydrofluoric acid content of the solution is converted to hydrofluosilicic acid by reaction with silica supplied thereto as at 33. The reaction mixture from vessel 31 passes by way of discharge conduit 34 onto a filter 35 where the excess silica is filtered out, as at 36, yielding a saleable, relatively concentrated, aqueous solution of hydrofluosilicic acid which can be passed to storage through line 37.

In the exploitation of this process it frequently will transpire that the values in the bottom sludge 41 in the bottom section 22 of the recycle still warrant the slight expense of their recovery. In such event, the bottom sludge—comprising a relatively concentrated sulphuric acid and metal sulphates, e.g. sulfates of manganese, iron and aluminum—is diverted through pipe 42, onto a filter 43 thereby recovering (a) a concentrated sulphuric acid recycle which is returned by conduit 44 to the recycle still and (b) a filter cake composed of the aforesaid metal sulfates in crystalline form. As has been noted in this specification, the metal sulphates can—if the same is so desired—be caused by known procedures to yield up their metal values.

Reverting to the "upgrading" aspect of the invention, I now describe my preferred specific procedure:

In carrying out the solubilizing (i.e., leaching step on raw ore), the leach solution (i.e., the "liquid phase" of the dissolving zone) should have an  $H_2SiF_6$  content of 10-15% by wt., and the free HF content (i.e., the recycled HF plus the make-up HF) per unit of raw ore should be about 10% by wt., more or less; and the solids in the resulting reaction mixture slurry should be from about 25 to about 30% by wt. The agitated reaction mixture should pass through the dissolving zone in from about 0.5 to about 3.0 hours time. The optimum temperature for the solubilizing step appears to be in the range 85-100° C.

Raw ore at minus 100 mesh ..... gm 50  
 30%  $H_2SiF_6$  ..... ml 75  
 50% HF ..... ml 10

and  
 70  $H_2O$  ..... ml 75

are slurried together and the slurry is heated to and maintained at about 95-100° C. for 30-50 minutes; the slurry then is filtered, and the separated phase is washed with water and dried.

The above procedure was used in processing the following specific examples, demonstrating the chemistry of the upgrading process.

| EXAMPLE I.—AMPA ORE (BRAZIL)   |                  |                        |
|--------------------------------|------------------|------------------------|
|                                | Raw Ore, Percent | Processed Ore, Percent |
| (a) Coarse Fraction:           |                  |                        |
| Mn                             | 52.6             | 58.0                   |
| Fe                             | 3.9              | .73                    |
| SiO <sub>2</sub>               | 1.37             | .07                    |
| Al <sub>2</sub> O <sub>3</sub> | 5.3              | 1.52                   |
| P                              | .069             | .063                   |
| MnO <sub>2</sub>               |                  | 86.8                   |
| (b) Fine Fraction:             |                  |                        |
| Mn                             | 50.1             | 58.3                   |
| P                              | .074             | .075                   |
| MnO <sub>2</sub>               | 71.7             | 87.1                   |

  

| EXAMPLE II.—COMOLOG ORE (GABON) |                  |                        |
|---------------------------------|------------------|------------------------|
|                                 | Raw Ore, Percent | Processed Ore, Percent |
| Mn                              | 53.2             | 58.9                   |
| Fe                              | 2.45             | .56                    |
| Al <sub>2</sub> O <sub>3</sub>  | 5.92             | 1.96                   |
| SiO <sub>2</sub>                | 1.86             | .105                   |
| P                               | .11              | .106                   |
| MnO <sub>2</sub>                | 79.3             | 90.5                   |
| Zn                              | .08              | .006                   |

  

| EXAMPLE III.—BELGIAN CONGO ORE |                  |                        |
|--------------------------------|------------------|------------------------|
|                                | Raw Ore, Percent | Processed Ore, Percent |
| Mn                             | 56.0             | 59.5                   |
| Fe                             | 1.2              | .5                     |
| Al <sub>2</sub> O <sub>3</sub> | 2.02             | 1.0                    |
| SiO <sub>2</sub>               | .68              | .08                    |
| P                              | .15              | .127                   |
| MnO <sub>2</sub>               | 83.16            | 88.7                   |
| Cu                             | .13              | .01                    |

  

| EXAMPLE IV.—IMMINI (MOROCCAN) ORE |                  |                        |
|-----------------------------------|------------------|------------------------|
|                                   | Raw Ore, Percent | Processed Ore, Percent |
| Mn                                | 54.2             | 58.1                   |
| MnO <sub>2</sub>                  | 84.6             | 90.1                   |

  

| EXAMPLE V.—URUCUM ORE (COARSE) |                  |                        |
|--------------------------------|------------------|------------------------|
|                                | Raw Ore, Percent | Processed Ore, Percent |
| Mn                             | 48.2             | 53.5                   |
| Fe                             | 9.4              | 3.6                    |
| P                              | .140             | .112                   |
| MnO <sub>2</sub>               | 70.6             | 81.4                   |

I have found it advisable, in the above-described upgrading operation, to use about 2.0 pounds of wash water for each 1.0 pound of ore product. When (as is highly desirable) the upgrading is integrated into a cyclic process, about 0.2-0.4 pound of this 2.0 pounds of  $H_2O$  will depart from the system in the form of a by-product 30% solution of  $H_2SiF_6$ , and somewhat less than this amount will depart in the sulfate sludge. Consequently, about 1.5 pounds of  $H_2O$  must be volatilized, for each 1.0 pound of upgraded ore produced, in the distilling, or fluorine-recovering, step of the completed cycle.

The "upgrading" realizable by the observance of the principles of the present invention is, in almost all cases, very surprisingly substantial in extent and of great technical advantage. This will be understood from a consideration of the extent of beneficiation which I have realized —by carrying out the process of this invention—on the ores mentioned in the above specific examples.

The upgraded  $MnO_2$  ore product of this process has been improved in a number of significant and important respects; the  $Mn^{+4}$  content has been increased; the inactive gangue—including iron—content has been minimized; the dioxide has been activated (resulting, in many cases, in producing a true “battery grade oxide” from a relatively poor ore unusable in a battery); and the oxidation potential of the  $MnO_2$  has been improved. This elevation of a non-battery grade to a battery grade ore by the carrying out of the present process is particularly striking in the processing of an ore of the gamma or rho crystalline type.

I claim:

1. Process of upgrading a manganese ore wherein a substantial part of the content of manganese-containing compounds consists of manganese dioxide, said ore containing a gangue constituent of the group consisting of compounds of Si, Al, Fe, P, Pb, Zn, Cu, Ca and Mg, which comprises treating the ore in particulate form with an aqueous solution of a dissolving agent of the group consisting of HF,  $H_2SiF_6$  and mixtures of HF and  $H_2SiF_6$  whereby to leach out such gangue constituents and separating the resulting aqueous phase from the solid phase.

2. Process of upgrading a manganese ore wherein a substantial part of the content of manganese-containing compounds consists of manganese dioxide, said ore containing a gangue constituent of the group consisting of compounds of Si, Al, Fe, P, Pb, Zn, Cu, Ca and Mg, which comprises treating the ore in particulate form with an aqueous solution of a dissolving agent of the group consisting of HF,  $H_2SiF_6$  and mixtures of HF and  $H_2SiF_6$  whereby to produce an upgraded  $MnO_2$  product and an aqueous mother liquor containing solubilized gangue constituents and fluorine values, separating said product from said liquor and recovering the fluorine values from said mother liquor.

3. The process defined in claim 2 characterized in that the same is a cyclical process in which at least a substantial part of the recovered fluorine values is recycled as the aqueous solution of dissolving agent.

4. Cyclic process of upgrading a manganese ore wherein a substantial part of the content of manganese-containing compounds consists of manganese dioxide, said ore including a gangue constituent of the group consisting of compounds of Si, Al, Fe, P, Pb, Zn, Cu, Ca and Mg, which comprises establishing a dissolving zone; feeding to the dissolving zone said ore in particulate form and an aqueous solution of  $H_2SiF_6$  and HF; continuously removing from said zone a slurry of leached ore and mother liquor; separating leached ore from mother liquor and washing the leached ore; adding the wash water to the mother liquor; returning part of the mother liquor to the dissolving zone; reacting the remainder of the mother liquor with  $H_2SO_4$ , at an elevated temperature at least as high as 160° C., thereby (a) forming sulfates of the soluble metal values of the mother liquor and (b) volatilizing the water and the fluorine values, the latter in the form of HF and  $SiF_4$ ; refluxing the resulting vapors under conditions to yield (1) a vapor phase consisting essentially of water; and (2) a liquid phase consisting essentially of a 30% aqueous solution of  $H_2SiF_6$  plus HF; returning a part of the resulting liquid phase to the dissolving zone; and removing the remainder of the liquid phase from the closed system.

5. Cyclic process of upgrading a manganese ore wherein a substantial part of the content of manganese-containing compounds consists of manganese dioxide, said ore including a gangue constituent of the group consisting of compounds of Si, Al, Fe, P, Pb, Zn, Cu, Ca and Mg, which comprises establishing a dissolving zone; feeding to the dissolving zone said ore in particulate form and an aqueous solution of  $H_2SiF_6$  and HF; continuously removing from said zone a slurry of leached ore and mother liquor; separating leached ore from the mother liquor and washing the leached ore; adding the wash water to the mother liquor; returning part of the mother liquor to the dissolving zone; reacting the remainder of the mother liquor with  $H_2SO_4$ , at an elevated temperature at least as high as 160° C., thereby (a) forming sulfates of the soluble metal values of the mother liquor and (b) volatilizing the water and the fluorine values, the latter in the form of HF and  $SiF_4$ ; refluxing the resulting vapors under conditions to yield (1) a liquid phase consisting essentially of a 15-43% aqueous solution of  $H_2SiF_6$  plus HF and (2) a vapor phase consisting essentially of water; returning a part of the resulting liquid phase to the dissolving zone; and treating the remainder of the liquid

phase from the refluxing operation with silica in an amount at least equal to the free HF content of said liquid phase, whereby to produce  $H_2SiF_6$  product.

6. Cyclic process of upgrading a manganese ore wherein a substantial part of the content of manganese-containing compounds consists of manganese dioxide, said ore including a gangue constituent of the group consisting of compounds of Si, Al, Fe, P, Pb, Zn, Cu, Ca and Mg which comprises establishing a dissolving zone; feeding to the dissolving zone said ore in particulate form and an aqueous solution of  $H_2SiF_6$  and HF; said dissolving agent containing from about 10 to about 15% by wt. of  $H_2SiF_6$  based on the solution and about 10% of total free HF (in recycled solution plus make-up addition) based on weight of raw ore, and the solids in the resulting slurry being from about 25 to about 30% by weight; continuously removing from said zone a slurry of leached ore and mother liquor; separating leached ore from the mother liquor and washing the leached ore; adding the wash water to the mother liquor; returning part of the mother liquor to the dissolving zone; reacting the remainder of the mother liquor with  $H_2SO_4$ , at an elevated temperature at least as high as 160° C., thereby (a) forming sulfates

of the soluble metal values of the mother liquor and (b) volatilizing the water and the fluorine values, the latter in the form of HF and  $SiF_4$ ; refluxing the resulting vapors under conditions to yield (1) a liquid phase consisting essentially of a 15-43% aqueous solution of  $H_2SiF_6$  plus HF and (2) a vapor phase consisting essentially of water; returning a part of the resulting liquid phase to the dissolving zone; and treating the remainder of the liquid phase from the refluxing operation with silica in an amount at least equal to the free HF content of said liquid phase, whereby to produce  $H_2SiF_6$  product.

#### References Cited

#### UNITED STATES PATENTS

|    |           |         |                  |       |        |
|----|-----------|---------|------------------|-------|--------|
| 15 | 2,584,894 | 2/1952  | MacIntire        | ----- | 23-88  |
|    | 2,724,646 | 11/1955 | Stringham et al. | ----- | 75-14  |
|    | 3,055,733 | 9/1962  | Land et al.      | ----- | 73-88  |
|    | 3,149,961 | 9/1964  | Moklebust        | ----- | 75-121 |

20 DAVID L. RECK, *Primary Examiner.*  
N. F. MARKVA, *Assistant Examiner.*